

## UNITED STATES PATENT OFFICE.

THURLOW W. MORGAN AND WILLIAM W. MURRAY, OF CHICAGO, ILLINOIS, ASSIGNEES  
TO CONTINENTAL CAN COMPANY, INC., OF NEW YORK, N. Y., A CORPORATION OF  
NEW YORK.

## PROCESS FOR PREVENTING DISCOLORATION OF CANNED FOODS.

No Drawing.

Application filed May 16, 1925. Serial No. 30,873.

To all whom it may concern:

Be it known that we, THURLOW W. MORGAN and WILLIAM W. MURRAY, citizens of the United States, residing at Chicago, in the county of Cook and State of Illinois, have invented new and useful Improvements in a Process for Preventing Discoloration of Canned Foods, of which the following is a specification.

10 The invention relates to new and useful improvements in a process for preventing discoloration of canned foods.

It is a well known fact that in the processing of many canned foods, there are formed 15 sulphur compounds, which occasionally react either during processing or subsequent thereto, with tin plate metal containers forming dark colored compounds, which are objectionable in appearance.

20 The present invention is directed to a process whereby the formation of such dark colored compounds are prevented.

Through a series of experiments with 25 processing foods in tin cans, it has been found that if an insoluble metallic compound of such metal or metals as form sulphides that are not dark colored such as zinc sulphide or cadmium sulphide, is thoroughly incorporated with the ingredients and homogeneously distributed through a lacquer prior to the application of the lacquer to the 30 surface of the tin plate, so that said compound becomes a component part of the lacquer, the discoloration referred to above is avoided. It has also been found that it 35 is not necessary to apply this lacquer bearing the insoluble metallic compound over the entire inner surface of the metal container, but if the ends of the container are thus 40 coated, the discoloration is avoided.

In carrying out the invention, an insoluble

metallic compound of the character specified above is ground to a very fine powder and from one to six per cent of such powder, is mixed with the ingredients forming the lacquer which is to be coated on the metal. By using such a fine powder, it may be so thoroughly incorporated with the ingredients as to become homogeneously distributed throughout the entire lacquer. The lacquer 45 is then prepared in the ordinary way and the sheets coated therewith. These coated sheets may be used in making the entire container, or may be used in making the ends 50 or bodies only of the container.

When the insoluble metallic compound is incorporated in the lacquer after the manner above described, it becomes permanently embodied in the lacquer and will be held in place on the inside of the container during 55 processing and subsequently thereto.

What we claim is—

The process of preventing the discoloration of canned foods comprising providing the inner surface or a portion thereof, of the 60 metal forming the container for the food, with a lacquer coating having an insoluble metallic compound of such metal or metals forming sulphides which are not dark colored thoroughly incorporated with the ingredients and homogeneously distributed through the lacquer prior to the application of the lacquer to the surface of the metal, so that said compound is permanently embodied in the lacquer and held in place on 65 the inside of the container during processing and subsequent thereto.

In testimony whereof we affix our signatures.

THURLOW W. MORGAN.  
WILLIAM W. MURRAY.